

## UNITED STATES PATENT OFFICE

CARL O. JOHNS, OF ELIZABETH, NEW JERSEY, ASSIGNOR TO STANDARD OIL DEVELOPMENT COMPANY, A CORPORATION OF DELAWARE

## LIQUID FUEL

No Drawing.

Application filed May 21, 1924. Serial No. 714,810.

This invention relates to motor fuels, and particularly motor fuels which it is desired shall be operable under relatively high engine-compressions without knocking or detonation.

As is well known, certain petroleum hydrocarbons are sensitive to high engine-compressions, and motor fuels containing such constituents are prone to knock or detonate when used in engines having compressions exceeding a relatively low ratio. To meet this condition it has been proposed to add to such fuels a metallo-alkyl compound, particularly lead tetraethyl. While effective in reducing the knocking propensities of the fuel, objection is made in some instances to the presence of as much lead as is involved in the amount of agent required.

In accordance with the present invention, the amount of lead or other metallo-alkyl compound necessary to accomplish the desired object can be minimized, it being found that in adding lead tetraethyl to gasoline for instance, the knocking propensity of the gasoline is reduced not in direct proportion with increasing increments of added lead tetraethyl but the first cubic centimeter of lead compound for instance per gallon of gasoline is the most effective while the result of additional increments of the anti-knock agent is successively less. In preparing a motor fuel, I employ a small amount of lead tetraethyl sufficient in quantity to produce the first and greatest effect but instead of adding further increments of lead tetraethyl to equal the total proportion of the agent heretofore customarily used, I further modify the petroleum hydrocarbons by the addition of a small proportion of an alcohol; as for example ethyl alcohol, methyl alcohol, or isopropyl alcohol or mixtures thereof. The alcohol may be added in amount of 3-10% to the petroleum hydrocarbons, and 1-2 cc. of lead tetraethyl may be added to the mixture. For example one advantageous composition comprises a mixture of about 95% of gasoline and 5% of ethyl alcohol, and 1½ cc. of lead tetraethyl per gallon of the mixture. By using my preferred type of modified fuel, I am able to materially decrease

the quantity of anti-knock agent needed in a gasoline to produce a fuel that may be used without detonation in internal combustion engines having relatively high compressions.

## I claim:

1. A motor fuel which comprises a mixture of about 95% of gasoline and 5% of ethyl alcohol, and lead tetraethyl in the amount of about 1½ cc. per gallon of the mixture. 55
2. A motor fuel which comprises a mixture of 90-97% of gasoline and 3-10% of an alcohol with a boiling point within the gasoline range, and lead tetraethyl in the amount of 1-2 cc. per gallon of the mixture. 60
3. A motor fuel which comprises a mixture of gasoline with not to exceed 10% of an alcohol with a boiling point within the gasoline range, and lead tetraethyl in amount not to exceed 2 cc. per gallon of the mixture. 65
4. A motor fuel which comprises a mixture of petroleum hydrocarbons with a relatively small proportion of an alcohol boiling within the range of said petroleum hydrocarbons, and lead tetraethyl in amount not to exceed 2 cc. per gallon of the mixture. 70
5. A motor fuel which comprises petroleum hydrocarbons, an alcohol boiling within the range of said hydrocarbons in relatively small proportion, and a metallo-alkyl anti-knock agent. 75

CARL O. JOHNS.

80

85

90

95

100